

Nov. 18, 1947.

G. J. GOEPFERT ET AL

2,431,035

ABRASIVE ARTICLES AND METHOD OF MAKING

Filed June 12, 1945

*Fig. 1.*



*Fig. 2.*



*Fig. 3.*



INVENTORS  
GEORGE J. GOEPFERT  
BY HALSEY W. BUELL

*W. J. Goepfert*  
Attorney

## UNITED STATES PATENT OFFICE

2,431,035

ABRASIVE ARTICLE AND METHOD OF  
MAKING

George J. Goepfert and Halsey W. Buell, Niagara Falls, N. Y., assignors to The Carborundum Company, Niagara Falls, N. Y., a corporation of Delaware

Application June 12, 1945, Serial No. 598,982

8 Claims. (Cl. 51—188)

1

This invention relates to endless abrasive belts formed from strips of flexible, abrasive coated web material. More particularly, it is concerned with the belt splice or joint formed by adhesively uniting the ends of the abrasive strip, and with the adhesive for uniting said ends. The invention is further pertinent to similar abrasive coated articles in which a continuous abrasive surface is obtained by adhesively joining contiguous ends of abrasive sheet material to form articles having endless abrading surfaces, such as cones, cylindrical drum covers and the like.

Endless abrasive belts and the like are commonly formed by adhesively splicing or joining the ends of a flexible, abrasive coated web material. The joint may be one of a number of different types, as for example, that formed by beveling a narrow area along each of the two ends, applying adhesive to the beveled areas and superimposing the upper and lower adhesive-coated beveled portions one on the other, and subjecting the assembly to pressure until the adhesive sets. Another form of belt joint or splice is obtained by skiving the end areas of the abrasive strip material free of abrasive, applying adhesive to the one abrasive-cleared area and to the underside of the abrasive-cleared area at the opposite end of the strip, overlapping the two ends, pressing together and allowing the adhesive to set. Regardless of the particular type of joint or splice employed, it is desirable to provide an adhesive therefor which will be quick-acting and also will result in a strong and flexible joint, and which is also satisfactory from the standpoint of stability, that is, an adhesive which will have a reasonably long, active adhesive life before subjecting to cure whereby it can be prepared for use and will remain stable and active adhesively for a prolonged period of time and will not have to be processed in a matter of a few hours after its preparation.

Hitherto, most abrasive belt failures have been the result of a defective or weak joint or splice. During the constant and repeated flexing of the belt joint in abrasive operations by the passage of the belt joint around the pulleys and under the work being ground, the belt joint has failed by a separation or delamination of the adhesively joined ends. Considerable effort has been directed to providing a belt joint which would be not only inexpensive and easily made, but which would have the requisite strength and flexibility to stand up under constant and repeated flexing action for the normal abrading life of the belt.

To accomplish the ends in mind, efforts heretofore have been directed to the use of more complicated joint structures. The bonding means employed having included such adhesives as animal and vegetable glues, latex, phenol formaldehyde resins and the like. The earlier glue adhesives are not of sufficient strength or flexibility and as a result a high percentage of them fail before the abrading life of the belt expires. While some improvement in strength has been obtained by the use of phenol formaldehyde resins and the like, and latex adhesives have resulted in somewhat higher flexibility, no belt joint has heretofore been found completely satisfactory in possessing the desired combination of behavior and properties. Moreover, certain difficulties of application, such as extended periods of cure, render the use of some adhesives undesirable or uneconomical.

More recently, it has been proposed to use certain urea aldehyde resin adhesive compositions as a bonding means in the joints of endless abrasive belts and like products. Although such compositions have been found satisfactory for use from the standpoint of rapidity of cure of the adhesive and the strength of the resulting joint, their use has been handicapped by the undesirable property such compositions have shown of instability upon standing. In other words, such urea aldehyde adhesive compositions when once prepared have had to be used within a relatively short time thereafter in order that the full strength of adhesion might be obtained. This deterioration in the adhesive characteristics of such compositions has been found to be a gradual one and consequently the ultimate strengths of belt joints embodying such adhesives have been undependable in that they varied from belt to belt with the result that many belt joints so made, after being accepted as of apparently adequate strength, have failed later under operating conditions.

It is therefore an object of the present invention to provide an improved belt splice which can be inexpensively and easily made, which will be of dependable high strength and will also obviate to a large degree the former difficulties and disadvantages encountered in belt splices and in the fabrication thereof under normal factory operating procedures.

In accordance with the present invention abrasive belt splices are formed in which the two abrasives cleared and beveled or skived termini of a flexible abrasive coated sheet or strip material are adhesively united by means of an inter-

venering coating of an adhesive comprising a urea aldehyde condensation product which has been modified by the inclusion therewith of a minor amount of a cure retardant such as furfuryl alcohol, together with a small amount of a suitable wetting agent. The use of plain urea aldehyde condensation products for such purposes is not desirable because of their inherent brittleness and lack of flexibility, and such use is not herein claimed. Also, certain modified urea aldehyde condensation products have been found unsuited for present purposes because of the instability of their adhesive activity and the consequent lack of dependability of abrasive belts and the like embodying them as the joining cements. However, it has been found that when urea aldehyde condensation products are properly stabilized by the inclusion of a suitable cure retardant such as furfuryl alcohol and a small percentage of a wetting agent such as that known and sold under the trade-mark "Tween" #20 therein, a belt joint is obtained which is uniform and dependable and has a high strength and flexibility and does not delaminate in use. Furthermore, the adhesive within the belt joint has a stability of adhesive action which permits of its use under normal factory operating conditions with a uniformity of result which provides dependability in the final products.

In order that the invention may be more clearly understood it will be described as it pertains to one particular type of belt splice which can be satisfactorily made in accordance with the invention, although it is not desired to limit the practice of the invention to the specific belt splice set forth and described in the drawing, in which

Figure 1 is a longitudinal, enlarged cross-section of the mating beveled ends of a belt, with adhesive coating, but prior to final splicing;

Figure 2 is a longitudinal, enlarged cross-section of a completed splice; and

Figure 3 is a top plan view of the completed splice shown in Figure 2.

Referring further to the drawing, the coated abrasive sheet or web material 2 is first slit into appropriate widths and then cut to length. This coated abrasive sheet material comprises a suitable flexible backing 3, such as paper or cloth, to which is adhesively secured a layer 4 comprising abrasive grains, such as granular aluminum oxide, silicon carbide, or other granular abrasive material, bonded to the backing 3 by any suitable adhesive substance, such as glue, resins, or the like, singly or in combination. The end or cross cut 5 is usually made at an angle to the lengthwise direction of the strip as shown in Figure 3, but this is not a limiting condition as the cut could be made normal to the lengthwise direction. In the actual preparation of the splice narrow areas at the ends of the abrasive-coated strip are beveled in the manner shown in Figures 1 and 2. The beveled surface 6 at one end of the abrasive strip is on the under side of the strip material and equal in area to the abrasive-cleared and beveled top surface area 7 at the opposite end of the abrasive strip. After the two ends have been skived and beveled, one or both of the beveled surfaces 6 and 7 are given a thin coating 8 of modified urea aldehyde condensation product containing furfuryl alcohol and a wetting agent. The beveled areas are then superimposed as shown in Figure 2 and subjected to pressure and heat to form the joint 9 in which the intervening

adhesive layer 8 serves to securely unite and hold the two ends in position.

Urea aldehyde adhesives which have been found to be highly satisfactory for belt joints have been obtained by modifying catalyzed urea aldehyde condensation products by the inclusion therewith of from 0.5 to 5% of furfuryl alcohol as a cure retarding agent together with the incorporation in the urea aldehyde condensation product of a small amount of a wetting agent. The addition of 0.5% of a wetting agent such as that known and sold under the trade-mark "Tween" #20 (which is a sorbitan monolaurate polyoxyalkylene derivative) has been found to give satisfactory results. Other wetting agents which may be used include those sold under the trade-marks "Aerosol" OT (dioctyl ester of sodium sulfo succinic acid), "Triton" W30 (a sulfated aromatic ether alcohol), "Span" 20 (sorbitan monolaurate), and "Tergitol" 08 (sodium salt of a higher secondary alkyl sulfate). The resulting reaction products produce belt joint adhesives of high stability in adhesive action so that the resulting adhesives can be employed to make dependable abrasive belt joints for as long as 48 hours or more after preparation of the adhesive. Moreover the above described adhesives provide joints of uniform high strength and flexibility capable of withstanding the constant flexing action encountered in the use of abrasive belts and like products wherein splices are essential.

The initial reaction products of a urea with a methylene-containing body are obtainable in the form of aqueous solutions or suspensions, which products when spread into a film and heated pass quickly and directly to the final, cured state and require temperatures and/or periods of cure substantially lower than those required to heat-harden the phenolic resins. They are obtainable in a considerable number of varieties, depending upon the specific urea compound employed, the relative proportion of the urea body and the methylene-containing body which are initially reacted, and the type of catalyst employed in bringing about the reaction. While our invention is not limited to any particular type of such resin, we have found that it is generally desirable to employ an initial reaction product which is not heat-hardening unless mixed with a separate liquid which acts as a catalyst and hardening agent for the reaction product and which matures quickly and directly to the final cured state when spread into a film, and to include a minor amount of furfuryl alcohol as a cure retardant to increase the adhesive stability of the cement, and a small amount of a wetting agent to increase the strength of adhesion of the cement to the cemented belt surfaces.

The usual urea condensation products are obtainable by reacting a urea such as thiourea or ordinary urea or mixtures thereof with a methylene-containing body such as formaldehyde, the formaldehyde probably being present in excess over that required to form dimethylol urea. Upon heating such mixture in the presence of either an acid or basic catalyst, it is generally believed that the latter product is obtained in colloidal form suspended in water. The reaction may be stopped by bringing the liquid to approximately the neutral point where it is neither acid nor alkaline. Such a product may then be made reactive by mixing with a suitable proportion of a hardening agent or catalyst which is of acidic nature or yields an acid reaction in solution or preferably a material which is normally basic

but ultimately becomes acidic. For example, the hardening agent may be prepared by dissolving urea or thiourea in water containing substantial proportions of ammonia and ammonium sulphate. Alternatively, ammonium thiocyanate may be substituted for at least part of the ammonium sulphate. In general, sulphur-containing compounds, such as an ammoniacal solution of ammonium sulphate in water, or in fact, an ammoniacal solution of any ammonium salt which will give an acid reaction in water, may be employed to bring about the reaction of the initial product to the final infusible condition. Various alkyl derivatives of ammonia may be used instead of ammonia in preparing the hardening agent. Such compounds have the advantage that the fumes evolved therefrom when the articles are heated are less objectionable than ammonia.

It has been further found that the ammoniacal solution of ammonium sulphate in water and the alkyl derivatives of ammonia which are used as catalysts or hardening agents for the urea condensation products can be replaced by certain organic materials such as organic phosphates and the like which are very satisfactory for the purpose. That material sold under the trademark "Bakelite" XK-15256 is a commercial organic phosphate available on the market and suitable for use as a hardener in practicing the present invention.

We have found that an improvement in the adhesive stability of urea aldehyde condensation product cements when used as the adhesive in endless abrasive belt joints and the like is obtained by the inclusion of from 0.5 to 5% of furfuryl alcohol in the adhesive composition as a cure retardant and stabilizer for the adhesive. The exact amount of cure retardant used will to some extent depend upon the amount and type of catalyst used in conjunction with the urea aldehyde condensation product. The further addition of a small amount of a wetting agent enhances the strength of adhesion of such adhesive composition to the belt surfaces being joined. We have been able, by the use of 1% furfuryl alcohol together with the use of 0.5% of a wetting agent such as "Tween" #20 (defined hereinabove) to provide a satisfactory high strength urea aldehyde adhesive composition in belt joints which has sufficient stability to remain adhesively active for longer than 48 hours. By contrast the urea aldehyde adhesives hitherto used for the purpose were unsatisfactory unless used the same day they were prepared.

The following specific examples are offered by way of illustration only, and given in detail the manner in which the invention is practiced and the nature of the adhesive used to form the belt joint.

*Example I*

Any suitable flexible, abrasive coated web material is first cut to the appropriate length and width and the ends of the resulting abrasive strip beveled and one end skived of abrasive in the manner previously set forth. The beveled areas are then coated with an adhesive consisting of:

Parts by weight

Liquid heat-hardenable urea-aldehyde condensation product, such as the urea-formaldehyde resin sold under the trade-mark "Bakelite" XRU-13108 100

urea-aldehyde condensation product containing 60% solids.

Parts by weight

|    |                                                                                                                                                   |     |
|----|---------------------------------------------------------------------------------------------------------------------------------------------------|-----|
| 5  | A hardening agent, such as that sold under the trade-mark "Bakelite" XK-12435 which consists of ammonium sulfate, thiourea and ammonium hydroxide | 10  |
| 10 | Furfuryl alcohol                                                                                                                                  | 1   |
| 15 | A wetting agent such as that sold under the trade-mark "Tween" #20 which consists of a sorbitan monolaurate polyoxyalkylene derivative            | 0.5 |
| 20 | Water                                                                                                                                             | 100 |

15 The adhesive-coated ends are then air- or force-dried, assembled and pressed in a warm clamp having a temperature of about 120° F. for 20 seconds, following which the joined parts are removed and clamped in a hot clamp having a temperature of about 300° F. for 20 seconds.

*Example II*

25 An abrasive belt joint was made as described in Example I except that in preparing the adhesive therefor the "Bakelite" XKU-12435 hardening constituent was replaced by "Bakelite" XK-14616 hardener, which consists of an ammonical solution of ammonium sulphate, containing 22% free ammonia and 10% ammonium sulphate.

30 It is not desired to be limited to the type of belt joint or splice shown, as the invention can be practiced with any type of splice where two abrasive coated strips or sheets are adhesively united to provide a continuous, flexible abrasive surface. For example, joints or splices can be made by skiving the abrasive from two end portions of an abrasive strip and overlapping the two cleared ends with a layer of intervening adhesive. Likewise V-shaped splices, or joints having various other configurations, can be made in which the furfuryl alcohol-modified urea condensation products as above set forth can be employed as the combining means to produce an improved splice. Likewise, the invention is not to be considered as limited to the specific adhesive compositions of the examples given.

35 In the claims we have used the word "urea" to include both ordinary urea and derivative or substitution products of urea, such as thiourea and the like.

40 Similarly, other forms of apparatus for applying heat and pressure other than the heated clamps set forth in the examples may be used, such as hot presses, mandrels or rolls.

45 While we have described our invention with particular reference to certain specific examples, it will be understood that other equivalent materials may be employed, together with other modifications and embodiments common to the art. The invention is therefore not to be restricted to the specific steps and materials herein described, but rather is to be considered as of the scope defined in the appended claims.

50 65 We claim:

1. An endless abrasive article of manufacture of flexible, abrasive-coated web material having a joint formed by two adhesively joined end portions, the adhesive of said joint comprising the 55 reaction product of a mixture comprising a major proportion of a urea aldehyde condensation product, a minor proportion of furfuryl alcohol, and a small amount of an organic wetting agent which depresses the surface tension of the adhesive with respect to the web material.

60 65 The urea resin is an aqueous suspension of a 70 75

2. An endless abrasive article of manufacture of flexible, abrasive-coated web material having a joint formed by two adhesively joined end portions, the adhesive of said joint comprising the reaction product of a mixture comprising a major proportion of a water-soluble urea aldehyde condensation product, a minor proportion of furfuryl alcohol, and a small amount of an organic wetting agent which depresses the surface tension of the adhesive with respect to the web material.

3. An endless abrasive article of manufacture of flexible, abrasive-coated web material having a joint formed by two adhesively joined end portions, the adhesive of said joint comprising the reaction product of a mixture comprising a water-soluble urea aldehyde condensation product, 0.5 to 5% furfuryl alcohol, and a small amount of an organic wetting agent which depresses the surface tension of the adhesive with respect to the web material.

4. An endless abrasive article of manufacture of flexible, abrasive-coated web material having a joint formed by two adhesively joined end portions, the adhesive of said joint comprising the reaction product of a mixture comprising a water-soluble urea aldehyde condensation product, approximately 1% furfuryl alcohol, and approximately 0.5% of an organic wetting agent which depresses the surface tension of the adhesive with respect to the web material.

5. An endless abrasive article of manufacture of flexible, abrasive-coated web material having a joint formed by two adhesively joined end portions, the adhesive of said joint comprising the reaction product of a mixture comprising a water-soluble urea aldehyde condensation product, approximately 1% furfuryl alcohol, and approximately 0.5% of a wetting agent such as a sorbitan monolaurate polyoxyalkylene derivative.

6. An endless abrasive article of manufacture of flexible, abrasive-coated web material having a joint formed by two adhesively joined end por-

tions, the adhesive of said joint comprising the reaction product of a mixture comprising a water-soluble, acid-catalyzed urea aldehyde condensation product, 0.5 to 5% of a cure retardant such as furfuryl alcohol, and approximately 0.5% of an organic wetting agent which depresses the surface tension of the adhesive with respect to the web material.

7. In the process of forming endless abrasive articles the step which comprises adhesively uniting the end portions of an abrasive sheet material by means of an intervening layer of an adhesive comprising a water-soluble urea aldehyde condensation product, 0.5 to 5% furfuryl alcohol, and a small amount of an organic wetting agent which depresses the surface tension of the adhesive with respect to the sheet material.

8. The method of forming endless abrasive articles which comprises removing the abrasive from an end of a flexible abrasive sheet, applying a liquid adhesive comprising a mixture of a water-soluble urea aldehyde condensation product, 0.5 to 5% of a cure retardant such as furfuryl alcohol, and a small amount of an organic wetting agent which depresses the surface tension of the adhesive with respect to the flexible sheet, to a terminal portion of the abrasive sheet, drying the liquid adhesive, overlapping the terminal portions with the adhesive therebetween, and applying heat and pressure to set the adhesive.

GEORGE J. GOEPFERT.  
HALSEY W. BUELL.

#### REFERENCES CITED

The following references are of record in the file of this patent:

#### UNITED STATES PATENTS

| Number    | Name               | Date          |
|-----------|--------------------|---------------|
| 2,350,861 | Argy et al. _____  | June 6, 1944  |
| 2,313,953 | Loughborough _____ | Mar. 16, 1943 |